# EUROPEAN PATENT SPECIFICATION

(11) **EP 2 373 771 B1**
(45) Date of publication and mention of the grant of the patent: **12.02.2014**
(21) Application number: 09830730.9
(22) Date of filing: 04.12.2009
(51) Int. Cl.: C10M 169/06, C10M 177/00, C10M 169/00, C10N 10/02, C10N 20/02, C10N 30/02, C10N 30/06, C10N 30/08, C10N 30/10, C10N 50/10, C10N 70/00

(54) **INDUSTRIAL AND AUTOMOTIVE GREASE AND PROCESS FOR ITS MANUFACTURE**
SCHMIERFETT FÜR INDUSTRIELLE UND KFZ-ANWENDUNG SOWIE VERFAHREN ZU SEINER HERSTELLUNG
GRAISSE INDUSTRIELLE ET AUTOMOBILE ET SON PROCÉDÉ DE FABRICATION

(30) Priority: 05.12.2008 US 200965 P
(43) Date of publication of application: 12.10.2011
(73) Proprietor: ExxonMobil Research and Engineering Company, Annandale, NJ 08801-0900 (US)
(72) Inventor: BARNES, Carol, A., Sarnia ON N7S 4V4 (CA); SMITH, Kamilah, N., Point Edward Ontario N7T 7W4 (CA); BLAHEY, Alan, G., Clearwater Ontario N&s 4l7 (CA); MACLAREN, Douglas, C., Petrolia Ontario N0N 1R0 (CA)
(74) Representative: Troch, Geneviève
(86) International application number: PCT/US2009/006387
(87) International publication number: WO 2010/065130

(56) References cited:
- EP-A2- 0 405 893
- WO-A1-2005/090531
- CA-A1- 996 537
- US-A1- 2004 178 118
- US-A1- 2004 209 787
- US-A1- 2006 100 292

## Description

### FIELD OF THE INVENTION

This invention relates to a lubricating grease composition suitable for industrial and automotive uses, and a process for its manufacture. In particular, the invention relates to a premium multipurpose grease composition exhibiting favorable water resistant properties, high and low temperature performance, and which is suitable for use in both industrial and automotive applications.

### BACKGROUND OF THE INVENTION

In North America and other northern climates, it is desirable for a lubricating grease to exhibit good performance over a wide range of temperatures. In addition, industrial greases often require good performance in wet environments. Testing methods and performance criteria established by the National Lubricating Grease Institute (NLGI) have become industry-wide accepted standards. These standards include greases for use in automotive applications. It is therefore desirable for lubricating grease to meet NLGI grade classification. Preferably, such greases should be multipurpose, being suitable for industrial applications and meet NLGI grade classification for automotive application.
For instance, WO 2005/090531 and EP 0 405 893 A2 disclose grease compositions having good water resistance.

There is a need to improve the water resistance and oxidation life of commercial premium greases that exhibit good high and low temperature performance. There is a further need to provide enhanced life expectancy and better overall performance in wet applications over current lubricants and improved performance in relation to low temperature torque and fretting wear. Accordingly, embodiments of this invention satisfy these needs.

### SUMMARY OF THE INVENTION

In one embodiment, this invention relates to a premium multipurpose lubricating grease suitable for industrial and automotive uses, and a process for making the same. In this embodiment, a lubricating grease composition is disclosed comprising, based on the overall grease composition:
(a) 30 to 40 wt% of at least one bright stock Group I oil;
(b) 5 to 15 wt% of at least one naphthenic group V oil,
(c) 5 to 10 wt% of at least one ISO 68 Group I oil,
(d) 20 to 30 wt% of at least one ISO 100 Group II oil;
(e) 2 to 6 wt% of a hydrophilic copolymer containing a styrene and a carboxylic acid, an anhydride or an ester; and
(f) 5 to 15 wt% of a soap thickener, and
(g) an antioxidant,
wherein the soap thickener (f) is dispersed into the at least one bright stock Group I oil (a) and the at least one naphthenic Group V oil (b) during a cooking phase and the at least one ISO 68 Group I oil (c) and the at least one ISO 100 Group II oil (d) are introduced during a finishing phase.
The present invention also provides such lubricating grease compositions as defined in any of accompanying claims 2 to 5.

In a second embodiment, a method for making a lubricating grease is disclosed. The method comprises: (a) obtaining at least one bright stock Group I oil, (b) obtaining at least one naphthenic Group V oil, (c) obtaining at least one ISO 68 Group I oil, (d) obtaining at least one ISO 100 Group II oil, (e) obtaining a hydrophilic copolymer containing a styrene and a carboxylic acid, an anhydride or an ester, (f) obtaining a soap thickener, (g) obtaining an antioxidant, and (h) mixing, based on the overall grease composition, 30 to 40 wt% of the at least one bright stock Group I oil (a), 5 to 15 wt% of the at least one naphthenic Group V oil (b), 5 to 10 wt% of the at least one ISO 68 Group I oil (c), 20 to 30 wt% of the least one ISO 100 Group II oil (d), 2 to 6 wt% of the polymer (e) 5 to 15 wt% of the soap thickener (f), and an antioxidant (g) to form a grease wherein the thickener (f) is dispersed into the at least one bright stock Group I oil (a) and the at least one naphthenic Group V oil (b) during a cooking phase and the at least one ISO 68 Group I oil (c) and the at least one ISO 100 Group II oil (d) are introduced during a finishing phase.

### BRIEF DESCRIPTION OF THE DRAWINGS

Fig. 1 is a graph illustrating the favorable low temperature torque properties of the inventive example over the comparative examples, as measured by ASTM D4693;
Fig. 2 is a graph illustrating the favorable fretting wear properties of the inventive example over the comparative examples, as measured by ASTM D4170;
Fig. 3 is a graph illustrating the favorable wheel bearing life properties of the inventive example over the comparative examples, as measured by ASTM D3527;
Fig. 4 is a graph illustrating the favorable water spray off properties of the inventive example over the comparative examples, as measured by ASTM D4049.

### DETAILED DESCRIPTION OF THE PREFERRED EMBODIMENTS

The present invention will be described in connection with its preferred embodiments.

In one embodiment, we have invented novel greases that are suitable for use in industrial applications, and at the same time meets NLG1 grade classification for use in automotive applications. The compositions of the greases and methods of manufacturing the greases are disclosed herein.

Various lubricating oils can be employed in preparing the grease compositions of the present invention. Applicants have found that using oils of a certain type during the cooking phase of the grease preparation, and oils of a different type during the finishing phase achieved a grease with favorable properties. Another embodiment of the present invention is the inclusion of a polymer that imparts excellent water resistance properties without compromising the low temperature performance of the grease. Applicants have found that using a hydrophilic polymer provided favorable properties.

Groups I, II, III, IV and V are broad categories of base oil stocks developed and defined by the American Petroleum Institute (API Publication 1509; www.API.org) to create guidelines for lubricant base oils. Group I base stocks generally have a viscosity index of between about 80 to 120 and contain greater than about 0.03% sulfur and/or less than about 90% saturates. Group II base stocks generally have a viscosity index of between about 80 to 120, and contain less than or equal to about 0.03% sulfur and greater than or equal to about 90% saturates. Group III stock generally has a viscosity index greater than about 120 and contains less than or equal to about 0.03 % sulfur and greater than about 90% saturates. Group IV includes polyalphaolefins (PAO). Group V base stocks include base stocks not included in Groups I-IV. Table 1 summarizes properties of each of these five groups.

**Table 1: Base Stock Properties**

| | Saturates | Sulfur | Viscosity Index |
|---|---|---|---|
| Group I | < 90% and/or | > 0.03% and | ≥ 80 and < 120 |
| Group II | ≥ 90% and | ≤ 0.03% and | ≥ 80 and < 120 |
| Group III | ≥ 90% and | ≤ 0.03% and | ≥ 120 |
| Group IV | Polyalphaolefins (PAO) | | |
| Group V | All other base oil stocks not included in Groups I, II, III, or IV | | |

The base stocks include at least one base stock of synthetic oils. Synthetic oil for purposes of this application shall include all oils that are not naturally occurring mineral oils.

In general, lubricating oils will typically comprise between 50 - 90 wt% of the overall grease composition. These oils will typically combine to provide an overall viscosity of the grease in the range of ISO 100 to ISO 320. The preferred viscosity for the present invention is between ISO 150 to ISO 275, with ISO 220 being the most preferred.

The lubricating oils used as the base stock in the cooking phase of the manufacturing process are at least one bright stock Group I oil and at least one naphthenic Group V oils. These oils will have a preferred viscosity in the range of 200 to 1400 cSt at 40°C, with a range of 200 to 500 cSt at 40°C being most preferred. A combination of heavy naphthenic oil and a bright stock are used as the base stock during the cooking phase, with 5-15 wt% heavy naphthenic oil and 30 - 40 wt% bright stock. The use of Group II oils during the cooking phase should be limited or avoided altogether. A combination of 5 - 10 wt% of an ISO 68 Group I and 20 - 30 wt% of an ISO 100 Group II are used during the finishing phase. Various other oils in smaller amounts may also be incorporated during the finishing phase.

The grease composition will also contain a soap thickener dispersed in the lubricating oil during the cooking phase to form a base grease. The soap thickener will comprise between 5% and 15% of the overall grease composition weight. The particular thickener employed is not critical and can vary broadly provided that it is effectively water insoluble. For example, the thickener may be based on aluminum, barium, calcium or lithium soaps, or their complexes. Soap thickeners may be derived from a wide range of animal oils, vegetable oils and greases, as well as the fatty acids derived therefrom. Carbon black, silica, and clays may be used as well as dyes, polyureas and other organic thickeners. Pyrrolidone-based thickeners can also be used. Preferred thickeners are based on lithium soap, calcium soap, their complexes, or mixtures thereof. Particularly preferred is a lithium or lithium complex thickener derived from reacting a C-18 fatty acid (12-hydroxy stearic acid) and a C-9 dicarboxylic acid (azelaic acid) with lithium hydroxide monohydrate. Canadian Patent 996537 provides a process for making this preferred thickener.

In one inventive embodiment, during the cooking phase of a preferred embodiment of the grease preparation, a mixture of Group I and Group V oils and a lithium soap of a C₁₂ to C₂₄ hydroxy fatty acid is first prepared. Then a C₂ to C₁₂ aliphatic carboxylic acid is added to that mixture and converted to its dilithium soap under conditions that are suitable for the formation of a complex between the lithium soap of the dicarboxylic acid and the lithium soap of the hydroxy fatty acid. While the lithium soap of the hydroxy fatty acid could be preformed and then dispersed in the lubricating oil medium, it is generally more expedient to prepare that soap in situ in the lubricating oil by neutralizing the hydroxy fatty acid with lithium base. The usual procedure during the cooking phase is to charge into the grease kettle the Group I and Group V oils and to then add the hydroxy fatty acid. The mixture of fatty acid and oil is heated sufficiently to bring about the dissolving action, e.g. at 82 to 93°C (180 to 200°F). Then a concentrated aqueous solution of the lithium base is added, usually in an amount slightly in excess of that required to neutralize the acid. The temperature at this stage of the cooking phase is usually between 93 to 99°C (200 and 210°F). The rate of addition of the lithium base may be varied. It is possible at this stage to proceed with the addition of the dicarboxylic acid and its subsequent neutralization to its dilithium soap, but this will require the neutraliztion to be conducted slowly or stepwise so as to ensure complexing of the two soaps with each other before the complete neutralization of the dicarboxylic acid has been brought about.
Accordingly, before proceeding with the addition of dicarboxylic acid and conversion to its dilithium soap, it is preferred that the temperature of the mixture of the Group I and Group V oils and lithium soap of the hydroxy fatty acid be raised to between 121 to 149°C (250 and 300°F). This is done in order to bring about a substantial dehydration of the mixture, such as, the removal of 70 to 100% of the water. As noted in Canadian Patent 996537, substantial dehydration at this stage also promotes the subsequent complexing reaction during the neutralization of the dicarboxylic acid. After substantial dehydration has been brought about, the mixture is cooled to between 110 to 116°C (230 and 240°F) and the dicarboxylic acid is added to the mixture. The mixture is stirred in order to bring about proper dispersion of the acid throughout the mixture and the concentrated aqueous solution of lithium base is then added to convert the dicarboxylic acid to its dilithium soap. Similarly with the neutralization of the fatty acid, the amount of lithium base added at this stage is slightly in excess of the amount required to neutralize both acid groups of the dicarboxylic acid. The temperature during this stage should preferably be maintained between 99 to 110°C 210 and 230°F), and more preferably between 104 to 110°C (220 to 230°F).

After all of the lithium base has been added to complete the neutralization of the dicarboxylic acid, the temperature of the grease mixture is once again raised in order to bring about dehydration. Preferably this will take place at 138 to 149°C (280 to 300°F). Following dehydration of the mixture, in order to ensure optimal thickener dispersion, the temperature of the mixture should further be raised to preferably between 193 to 204°C (380 and 400°F). The soap stock is then cooled during the finishing phase of the grease preparation. Finishing oils, including Group II oils and various other lubricating oils, may be added into the mixture at this point. Mixing may continue until the grease has reached ambient temperatures. When the temperature has been lowered to about 65°C (150°F), other grease additives can be introduced as would be understood by persons skilled in the art.

As mentioned previously, one embodiment contemplates the inclusion of a polymer. Various polymers may be used in greases, although the precise impact of any given polymer on a given grease cannot be predicted. Applicants have found that the use of a hydrophilic copolymer was important in achieving excellent water resistance properties. In a preferred embodiment of the present invention, maleic anhydride styrene esterified copolymer is used, with the preferred amount being between 2 and 6 wt% of the overall grease. The polymer may be incorporated during either the cooking phase or finishing phase of the grease preparation.

The preferred styrene maleic anhydride ester (SMAE) copolymer is unique from other polymer examples because it contains oxygen groups. The structure of the SMAE copolymer (shown below) has exposed hydroxyl and carbonyl groups that can act as hydrogen bond donors (former) and acceptors (latter). As a result, the SMAE copolymer is more hydrophilic than strictly hydrocarbon-based copolymers such as styrene isoprene and styrene isobutylene.

Equation 1 shows the chemical structure of the SMA ester and the esterification of styrene maleic anhydride copolymer to form a SMA ester and the resulting chemical structure of the SMA ester. The grease structure is a type of soap. The ability of the soap to dissolve in waters varies. Preferably, the grease soap should not readily dissociate in contact with water.

The grease soap structure is held together with a variety of bonds, including ionic bonds with the metal, hydrogen bonds within the oxygen-rich triglyceride and the ester function of 12-hydroxy stearic acid (once incorporated into the structure) and van der Waals interactions between the C-C side chains. When a grease is exposed to water, bond networks may be disrupted and the grease's structural stability may be compromised. This can result in poor performance in water resistance tests.

A polymer that incorporates or binds water molecules into its structure may enhance the water resistance performance of a grease. Hydrogen bonding capability present in certain copolymers. For example, SMAE can improve their ability to incorporate or bind water molecules into their respective structures. The water resistance performance of a grease may be improved where the copolymer provides preferential binding of the water, such as, the attraction of water to the copolymer, through hydrogen bonding, is stronger than the attraction of water to the grease structure.

The grease may also contain small amounts of supplemental additives, which include antioxidants, anti-wear agents and other additives. Specific antioxidants employed are not critical and can vary broadly to achieve favorable properties. A combination of a Group II oil and diphenylamine antioxidant was found to enhance the oxidation life of the grease, while achieving good high temperature performance. Antioxidants will typically comprise less than 5 wt% of the overall grease composition. The total amount of all additives, including the antioxidant, will typically be between 2 - 10wt% of the overall grease. A person skilled in the art will recognize the benefits of adding specific additives to the grease disclosed herein to achieve favorable properties.

This invention will be further understood by reference to the following tables and examples, which describes the preferred embodiment of the "Invention". Figures 1 through 4, collectively, illustrate the better overall performance of the inventive example 1 over the comparative examples with respect to low temperature torque, fretting water, wheel bearing life, and water spray off. The data, illustrated in bar chart form in the figures, is shown in chart form in Table 2 below.

### Examples

The examples in table 2 below disclose various screening tests for the influence of the base oils and thickener on overall grease performance. The grease performance tests include water spray-off, low temperature torque, fretting wear and wheel bearing life.

The results in Table 2 demonstrate that changes to the oils in either the cooking phase or the finishing phase will not yield a grease meeting all of the necessary NLGI performance criteria for automotive use.

**Table 2**

| **EXAMPLE #** | 1* | 2 | 3 | 4 | 5 | 6 |
|---|---|---|---|---|---|---|
| **BATCH #** | Invention 12-52-07 IP2007455 | 8 IP2007281/ GR1004-152 | B IP2007193 | 9 IP2007279/ GR1004-158 | 13-3 IP2007443 | 11-01-07 IP2007411 |
| **TOTAL BASE OILS** | | | | | | |
| ISO 100 Group II | 24 | 0 | 43.5 | 36.4 | 33.3 | 27.8 |
| Heavy Naphthenic | 10.2 | 11.7 | 0 | 7.8 | 10.4 | 32.9 |
| ISO 68 Group I | 8.7 | 16.6 | 0 | 0 | 0 | 0 |
| Bright Stock | 35.6 | 47.5 | 30.3 | 32.3 | 33.5 | 17.1 |
| ISO 22 Naphthenic | 0 | 4.1 | 0 | 0 | 0 | 0 |
| Kinematic Viscosity@40°C, cst | 206 | 238 | 185 | 211 | 223 | 201 |
| VI | 93 | 91 | 98 | 94 | 93 | 79 |
| Aniline Pt, °C | 119 | 115 | 125 | 122 | 122 | 112 |

| **COOK OILS** | | | | | | |
|---|---|---|---|---|---|---|
| ISO 100 Group II | 0 | 0 | 43.5 | 35.9 | 0 | 0 |
| Heavy Naphthenic | 10.2 | 11.7 | 0 | 7.8 | 10.4 | 32.9 |
| ISO 68 Group I | 0 | 11.8 | 0 | 0 | 0 | 0 |
| Bright Stock | 31.7 | 13.2 | 0 | 0 | 33.5 | 11.9 |
| ISO 22 Naphthenic | 0 | 4.1 | 0 | 0 | 0 | 0 |
| Kinematic Viscosity@40°C. cst | 405 | 163 | 104 | 123 | 440 | 306 |
| VI | 89 | 83 | 99 | 92 | 89 | 60 |
| Aniline Pt, °C | 119 | 107 | 124 | 119 | 120 | 102 |
| **FINISHING OILS** | | | | | | |
| ISO 100 Group II | 24 | 0 | 0 | 0.9 | 33.3 | 27.8 |
| Heavy Naphthenic | 0 | 0 | 0 | 0 | 0 | 0 |
| ISO 68 Group I | 8.7 | 4.8 | 0 | 0 | 0 | 0 |
| Bright Stock | 3.9 | 34.3 | 30.3 | 32.3 | 0 | 5.2 |
| ISO 22 Naphthenic | 0 | 0 | 0 | 0 | 0 | 0 |
| Kinematic Viscosity@40°C, cst, calc | 105 | 350 | 183 | 448 | 104 | 128 |
| Aniline Pt,°C, calc | 120 | 124 | 125 | 127 | 124 | 125 |

| **ADDITIVES** | | | | | | |
|---|---|---|---|---|---|---|
| Antioxidant (diphenylamine) | 1.5 | 1.5 | 1.5 | 1.5 | 1.5 | 1.5 |
| Polymer A | 3 | 3 | 3 | 3 | 3 | 3 |
| Polymer B | 0 | 0 | 0 | 0 | 0 | 0.3 |

| **PERFORMANCE** | | | | | | |
|---|---|---|---|---|---|---|
| Water Spray-off, D4049, wt% (35 max.) | 26 | 31 | 37 | 67 | 35 | 21 |
| Low Temp Torque, D4693, n-m (15.5 max.) | 11.4 | 11.9 | 8.2 | 9.8 | 9.6 | 17.2 |
| Fretting Wear, D4170, mg (10 max.) | 8.5 | 20.3 | 20.3 | 25.7 | 15 | 21 |
| Wheal Bearing Life, D3527, hr (125 min.) | 153 | 47 | | 130 | | 150 |

| | | | | | | |
|---|---|---|---|---|---|---|
| * Examples according to the invention | | | | | | |

Table 3 below discloses screening test for the influence of the polymer selection and concentration on overall grease performance. These tests includes water spray-off, wet roll, water washout, low temperature torque, fretting wear, wheel bearing life and apparent viscosity.

The results in Table 3 demonstrate that using 3 wt% Polymer A or maleic anhydride styrene ester copolymer exhibits excellent water resistance performance and also meets the other key performance parameters.

| **Legend 3a (Base Oil)** | | | **Legend 3a (Base Oil)** | |
|---|---|---|---|---|
| **Base Oil** | **Typical viscosity @ 40°C, cSt** | | **Polymer** | **Polymer type** |
| ISO 100 Group II | 100 | | Polymer A | maleic anhydride styrene ester copolymer |
| Heavy Naphthenic | 290 - 390 | | Polymer B | styrene isobutylene copolymer |
| ISO 68 Group I | 68 | | Polymer C | hydrogenated styrene-isoprene copolymer |
| Bright Stock | 480 | | Polymer D | hydrogenated styrene-isoprene star copolymer |
| ISO 100 Group I | 100 | | Polymer E | functionalized olefin copolymer |

Table 4 discloses screening tests for the influence of various antioxidants on grease performance for wheel bearing life. The results of Table 4 demonstrate that a combination of an ISO 100 Group II base oil and a diphenylamine antioxidant achieved good high temperature performance and oxidation life.

**Table 4**

| **EXAMPLE #** | **1*** | **19*** | **20*** | **21** | **22** |
|---|---|---|---|---|---|
| **BATCH #** | **Invention 12-52-07** | **GR1004-156-2** | **GR1004-156-3** | **GR1004-156-1** | **Batch 8 GR1004-152** |
| **BASE OILS** | | | | | |
| ISO 100 Group II | 24 | 24 | 24 | 24 | 0 |
| Heavy Naphthenic | 10.2 | 10.2 | 10.2 | 10.2 | 11.7 |
| ISO 68 Group I | 8.7 | 8.7 | 8.7 | 8.7 | 16.6 |
| Bright Stock | 35.6 | 35.6 | 35.6 | 35.6 | 47.5 |
| ISO 22 Naphthenic | 0 | 0 | 0 | 0 | 4.1 |

| **ADDITIVES** | | | | | |
|---|---|---|---|---|---|
| Polymer A | 3 | 3 | 3 | 3 | 3 |
| Antioxidant (diphenylamine) | 1.5 | 0.76 | 0.30 | 0 | 1.5 |

| **PERFORMANCE** | | | | | |
|---|---|---|---|---|---|
| Wheel Bearing Life, D3527, hr (125 min.) | 153 | 134 | 130 | 80 | 47 |

| LEGEND | | | | | |
|---|---|---|---|---|---|
| Base Oil | Typical viscosity @ 40°C, cSt | | | | |
| ISO 100 Group II | 100 | | | | |
| Heavy Naphthenic | 290-390 | | | | |
| ISO 68 Group I | 60 | | | | |
| Bright Stock | 480 | | | | |
| ISO 22 Naphthenic | 20 | | | | |

| | | | | | |
|---|---|---|---|---|---|
| * Examples according to the invention | | | | | |

## Claims

1. A lubricating grease composition comprising, based on the overall grease composition:
(a) 30 to 40 wt% of at least one bright stock Group I oil;
(b) 5 to 15 wt% of at least one naphtenic Group V oil,
(c) 5 to 10 wt% of at least one ISO 68 Group I oil;
(d) 20 to 30 wt% of at least one ISO 100 Group II oil;
(e) 2 to 6 wt% of a hydrophilic copolymer containing a styrene and a carboxylic acid, an anhydride or an ester;
(f) 5 to 15 wt% of a soap thickener, and
(g) an antioxidant,
wherein
the soap thickener (f) is dispersed into the at least one bright stock Group I oil (a) and the at least one naphthenic Grop V oil (b) during a cooking phase and
the at least one ISO 68 Group I oil (c) and the at least one ISO 100 Group II oil (d) are introduced during a finishing phase.

2. The grease in claim 1, where the copolymer is styrene maleic anhydride ester.

3. The grease in any one of the preceding claims, wherein the thickener is derived from reacting a mixture of a C₁₂ to C₂₄ hydroxy fatty acid and a C₂ to C₁₂ dicarboxylic acid with a lithium base.

4. The grease in claim 1, where the antioxidant is an amine-based antioxidant.

5. The grease in claim 1, where the antioxidant is diphenylamme.

6. A method for making a lubricating grease, said method comprising.
(a) obtaining at least one bright stock Group I oil;
(b) obtaining at least one naphthenic Group V oil;
(c) obtaining at least one ISO 68 Group I oil;
(d) obtaining at least one ISO 100 Group II oil;
(e) obtaining a hydrophilic copolymer containing a styrene and a carboxylic acid, an anhydride or an ester;
(f) obtaining a soap thickener;
(g) obtaining an antioxidant; and
(h) mixing, based on the overall grease composition, 30 to 40 wt% of the at least one bright stock (a), 5 to 15 wt% of the at least one naphthenic oil (b), 5 to 10 wt% of the at least one ISO 68 Group I oil (c), 20 to 30 wt% of the least one ISO 100 Group II oil (d), 2 to 6 wt% of the polymer (e), 5 to 15 wt% of the soap thickener (f), and the antioxidant (g) to form a grease wherein
the thickener (f) is dispersed into the at least one bright stock Group I oil (a) and the at least one naphthenic Group V oil (b) during a cooking phase and
the at least one ISO 68 Group I oil (c) and the at least one ISO 100 Group II oil (d) are introduced during a finishing phase.

## Patentansprüche

1. Schmierfettzusammensetzung, die, bezogen auf die gesamte Fettzusammensetzung:
(a) 30 bis 40 Gew.-% mindestens eines Bright Stock - Gruppe I Öls;
(b) 5 bis 15 Gew.-% mindestens eines naphthenischen Gruppe V Öls;
(c) 5 bis 10 Gew.-% mindestens eines ISO 68 Gruppe I Öls,
(d) 20 bis 30 Gew.% mindestens eines ISO 100 Gruppe II Öls;
(e) 2 bis 6 Gew.-% hydrophiles Copolymer, das ein Styrol und Carbonsäure, Anhydrid oder Ester enthält;
(f) 5 bis 15 Gew.-% Seifenverdicker und
(g) Antioxidans
umfasst;
wobei
der Seifenverdicker (f) in dem mindestens einen Bright Stock Gruppe I Öl (a) und dem mindestens einen naphthenischen Gruppe V Öl (b) während einer Kochphase dispergiert wird, und
das mindestens eine ISO 68 Gruppe I Öl (c) und das mindestens eine ISO 100 Gruppe II Öl (d) während einer Endbehandlungsphase eingeführt werden.

2. Fett nach Anspruch 1, bei dem das Copolymer Styrol/Maleinsäureanhydridester ist.

3. Fett nach einem der vorhergehenden Ansprüche, bei dem der Verdicker sich von der Umsetzung einer Mischung einer C₁₂-bis C₂₄-Hydroxyfettsäure und einer C₂- bis C₁₂-Dicarbonsäure mit einer Lithiumbase ableitet.

4. Fett nach Anspruch 1, bei dem das Antioxidans ein auf Amin basierendes Antioxidans ist.

5. Fett nach Anspruch 1, bei dem das Antioxidans Diphenylamin ist.

6. Verfahren zur Herstellung eines Schmierfetts, wobei das Verfahren umfasst:
(a) Bereitstellen mindestens eines Brigth Stock Gruppe I Öls,
(b) Bereitstellen mindestens eines naphthenischen Gruppe V Öls,
(c) Bereitstellen mindestens eines ISO 68 Gruppe I Öls,
(d) Bereitstellen mindestens eines ISO 100 Gruppe II Öls,
(e) Bereitstellen eines hydrophilen Copolymers, das ein Styrol und Carbonsäure, Anhydrid oder Ester enthält,
(f) Bereitstellen eines Seifenverdickers,
(g) Bereitstellen eines Antioxidans und
(h) Mischen, bezogen auf die Gesamtfettzusammensetzung, von 30 bis 40 Gew.-% des mindestens einen Brigth Stock (a), 5 bis 15 Gew.-% des mindestens einen naphthenischen Öls (b), 5 bis 10 Gew.-% des mindestens einen ISO 68 Gruppe I Öls (c), 20 bis 30 Gew.-% des mindestens einen ISO 100 Gruppe II Öls (d), 2 bis 6 Gew.-% des Polymers (e), 5 bis 15 Gew.-% des Seifenverdickers (f) und des Antioxidans (g) um ein Fett zu bilden, wobei
der Verdicker (f) in dem mindestens einen Brigth Stock Gruppe I Öl (a) und dem mindestens einen naphthenischen Gruppe V Öl (b) während einer Kochphase dispergiert wird und
das mindestens eine ISO 68 Gruppe I Öl (c) und das mindestens eine ISO 100 Gruppe II Öl (d) während einer Endbehandlungsphase eingeführt werden.

## Revendications

1. Composition de graisse lubrifiante comprenant, par rapport à la composition de graisse dans son ensemble :
(a) 30 à 40 % en poids d'au moins une huile de base lubrifiante de haute viscosité du Groupe I ;
(b) 5 à 15 % en poids d'au moins une huile naphténique du Groupe V,
(c) 5 à 10 % en poids d'au moins une huile ISO 68 du Groupe I ;
(d) 20 à 30 % en poids d'au moins une huile ISO 100 du Groupe II ;
(e) 2 à 6 % en poids d'un copolymère hydrophile contenant un styrène et un acide carboxylique, un anhydride ou un ester ;
(f) 5 à 15 % en poids d'un épaississant de type savon, et
(g) un antioxydant,
dans laquelle
l'épaississant de type savon (f) est dispersé dans la au moins une huile de base lubrifiante de haute viscosité du Groupe I (a) et la au moins une huile naphténique du Groupe V (b) pendant une phase de cuisson et la au moins une huile ISO 68 du Groupe I (c) et la au moins une huile ISO 100 du Groupe II (d) sont introduites pendant une phase de finition.

2. Graisse selon la revendication 1, dans laquelle le copolymère est un ester de styrène-anhydride maléique.

3. Graisse selon l'une quelconque des revendications précédentes, dans laquelle l'épaississant est obtenu par réaction d'un mélange d'un hydroxyacide gras en C₁₂ à C₂₄ et d'un diacide carboxylique en C₂ à C₁₂ avec une base au lithium.

4. Graisse selon la revendication 1, dans laquelle l'antioxydant est un antioxydant à base d'amine.

5. Graisse selon la revendication 1, dans laquelle l'antioxydant est la diphénylamine.

6. Procédé de fabrication d'une graisse lubrifiante, ledit procédé comprenant les étapes consistant à :
(a) obtenir au moins une huile de base lubrifiante de haute viscosité du Groupe I ;
(b) obtenir au moins une huile naphténique du Groupe V ;
(c) obtenir au moins une huile ISO 68 du Groupe I ;
(d) obtenir au moins une huile ISO 100 du Groupe II ;
(e) obtenir un copolymère hydrophile contenant un styrène et un acide carboxylique, un anhydride ou un ester ;
(f) obtenir un épaississant de type savon ;
(g) obtenir un antioxydant ; et
(h) mélanger, par rapport à la composition de graisse dans son ensemble, 30 à 40 % en poids de la au moins une base lubrifiante de haute viscosité (a), 5 à 15 % en poids de la au moins une huile naphténique (b), 5 à 10 % en poids de la au moins une huile ISO 68 du Groupe I (c), 20 à 30 % en poids de la au moins une huile ISO 100 du Groupe II (d), 2 à 6 % en poids du polymère (e), 5 à 15 % en poids de l'épaississant de type savon (f), et l'antioxydant (g) pour former un graisse, dans lequel
l'épaississant (f) est dispersé dans la au moins une huile de base lubrifiante de haute viscosité du Groupe I (a) et la au moins une huile naphténique du Groupe V (b) pendant une phase de cuisson et
la au moins une huile ISO 68 du Groupe I (c) et la au moins une huile ISO 100 du Groupe II (d) sont introduites pendant une phase de finition.
